

# United States Patent [19]

Battersby et al.

[11] 3,980,450

[45] Sept. 14, 1976

[54] **GASOLINE COMPOSITION**

[75] Inventors: **John Battersby, Frimley; Eric Simon Forbes, Lightwater, both of England**

[73] Assignee: **The British Petroleum Company Limited, London, England**

[22] Filed: **Aug. 5, 1974**

[21] Appl. No.: **494,710**

**Related U.S. Application Data**

[62] Division of Ser. No. 408,575, Oct. 23, 1973.

[30] **Foreign Application Priority Data**

Oct. 27, 1973 United Kingdom..... 49573/73

[52] **U.S. Cl. .... 44/72**

[51] **Int. Cl.<sup>2</sup> .... C10L 1/22**

[58] **Field of Search..... 44/72**

[56]

**References Cited**

**UNITED STATES PATENTS**

|           |         |             |       |
|-----------|---------|-------------|-------|
| 3,478,096 | 11/1969 | Cyba.....   | 44/74 |
| 3,637,358 | 1/1972  | Cyba.....   | 44/72 |
| 3,849,083 | 11/1974 | Dubeck..... | 44/72 |

*Primary Examiner*—Allen B. Curtis

*Assistant Examiner*—Y. Harris-Smith

*Attorney, Agent, or Firm*—Morgan, Finnegan, Pine, Foley & Lee

[57]

**ABSTRACT**

A carburettor detergent comprises a compound formula  $R-O-R^1-N.R^2.R^3$  where R is a hydrocarbyl group containing at least 20 carbon atoms,  $R^1$  is a hydrocarbyl or amino substituted hydrocarbyl group and  $R^2$  and  $R^3$  are hydrogen or an alkyl group.

**4 Claims, No Drawings**



carburettor is rated visually for deposits and rated on an arbitrary 0 to 10 scale, 10 indicating a clean carburettor.

The following results were obtained.

of isobutylene, R<sup>1</sup> is a polymethylene group containing 2 to 6 carbon atoms interrupted by an imino group, and R<sup>2</sup> and R<sup>3</sup>, which may be the same or different are hydrogen atoms or alkyl groups.

| Compound                                                                                                        | Concen-<br>tration<br>(ppm) | % N  | Rating |
|-----------------------------------------------------------------------------------------------------------------|-----------------------------|------|--------|
| None                                                                                                            | —                           | —    | 2.5-3  |
| PIB - O CH <sub>2</sub> CH <sub>2</sub> NH CH <sub>2</sub> CH <sub>2</sub> NH <sub>2</sub>                      | 140                         | 0.84 | 7.5    |
| PIB - O CH <sub>2</sub> CH <sub>2</sub> NH CH <sub>2</sub> CH <sub>2</sub> CH <sub>2</sub> N<br>CH <sub>3</sub> | 130                         | 0.97 | 7.5    |

We claim:

1. A fuel composition comprising gasoline and up to 1,000 parts per million of a carburettor detergent of the formula:



wherein R is a hydrocarbyl group containing from 20 to 500 carbon atoms and derived from the polymerization

2. A composition according to claim 1 wherein R<sup>2</sup> and R<sup>3</sup>, when alkyl groups, contain 1 to 4 carbon atoms.

3. A composition according to claim 1 which contains 50-200 parts per million of the carburetor detergent compound.

4. A composition according to claim 1 wherein R<sup>1</sup> is selected from the group consisting of —CH<sub>2</sub>CH<sub>2</sub>NH CH<sub>2</sub>CH<sub>2</sub>— and —CH<sub>2</sub>CH<sub>2</sub>CH<sub>2</sub>NHCH<sub>2</sub>CH<sub>2</sub>CH<sub>2</sub>—.

\* \* \* \* \*

30

35

40

45

50

55

60

65